

## 1

3,679,350

**PROCESS FOR THE DYEING OF TEXTILE MATERIALS MADE FROM MIXTURES OF POLYESTER AND CELLULOSIC FIBRES**

Rudolf Lowenfeld, Buchschlag, and Hans Kaiser, Offenbach am Main, Germany, assignors to Farbwerke Hoechst Aktiengesellschaft vormals Meister Lucius & Bruning, Frankfurt am Main, Germany

No Drawing. Filed May 6, 1970, Ser. No. 35,301  
Claims priority, application Germany, May 14, 1969,

P 19 24 803.4

Int. Cl. D06p 3/82

U.S. Cl. 8-21 C

6 Claims

**ABSTRACT OF THE DISCLOSURE**

Process for the semi-continuous or continuous dyeing of textile material made from mixtures of polyester and cellulosic fibres, the polyester fibre portion of which having been predyed with disperse dyestuffs, by impregnating said textile material with an alkaline solution containing a coupling component and a diazoamino or tetrazoamino compound or an anti-diazotate, as well as wetting and dispersing agents, and subsequently treating the textile material, without intermediate drying, with an acidic solution at temperatures of from 50° to 80° C. to achieve development of the dyestuff on the fibre.

The present invention relates to a new process for the dyeing of textile material made from mixtures of polyester and cellulosic fibres.

It is known that textile material made from mixtures of polyester and cellulosic fibres can be dyed to yield fast shades by using disperse dyestuffs and water-insoluble azo dyestuffs, the latter being produced on the fibre. The procedure is as follows: At first, the polyester fibre portion of the goods is dyed with disperse dyestuffs, either at boiling temperature and in the presence of dyeing accelerators, or under the conditions of the high-temperature dyeing method, or according to the Thermosol process; subsequently the water-insoluble azo dyestuff is produced on the cellulosic fibre portion by impregnation of the textiles with a coupling component and thereafter development of the dye with a diazotized aromatic amine. This process yields dyeings of good quality, but it needs much time and work, since the disperse dyestuff, the coupling component and the diazotized aromatic amine have to be applied in different dyeing baths.

A further well-known process is the following: The textile material is impregnated with an alkaline solution containing a coupling component, a diazoamino compound, a disperse dyestuff as well as a compound splitting off acids when heated. After drying the textiles, formation of the water-insoluble azo dyestuff on the cellulosic fibre portion is caused at temperatures of from 180° to 210° C., at the same time the disperse dyestuff is fixed on the polyester fibre portion, and finally, an alkaline after-treatment is carried out. This process is a very economic one, but its drawback resides in the fact that not all disperse dyestuffs are stable towards the high alkali quantities in the impregnation bath and that in an alkaline medium

## 2

many disperse dyestuffs are not completely fixed on polyester fibres. On the other hand, also the development of the water-insoluble azo dyestuff is not complete under the conditions of dry heat fixation, so that the colour yield is insufficient and the dyeings show considerably duller shades in comparison to those achieved by the way of a wet development. Further, this process requires an addition of urea, which may cause trouble in industrial practice on account of its annoying smell during the treatment with dry heat.

It has now been found that the aforesaid drawbacks in the dyeing of textile material made from mixtures of polyester and cellulosic fibres can be eliminated by impregnating said textile material, the polyester portion of which having been predyed with disperse dyestuffs, with an alkaline solution containing a coupling component and a diazoamino or tetrazoamino compound or an anti-diazotate, as well as wetting or dispersing agents, and subsequently treating it, without intermediate drying, with an aqueous solution of an acidic agent at temperatures of from about 50° to 80° C. in order to develop the azo dyestuff on the fibre.

The process of the invention is carried out as follows: The textile material, for example mixed fabrics made from polyester and cellulosic fibres, the polyester fibre portion of which having been dyed at first with a disperse dyestuff in known manner by impregnation, drying and subsequent heat fixation, is impregnated with an alkaline solution containing a coupling component and a diazoamino compound, a tetrazoamino compound or an anti-diazotate, as well as wetting or dispersing agents, then squeezed out and wound on a roller. The alkali content of the impregnation bath has to be kept at a level that keeps the coupling component from precipitation during the impregnation operation which is carried out at temperatures of from 30° to 60° C. The textile material has to be squeezed off thoroughly after its impregnation in order to obtain a very low liquor pick-up of the mixed fabric. After winding up the squeezed goods and dwelling them at room temperature of a slightly elevated temperature for a short time to allow for absorption of the coupling component by the fibre, or after an air-passage of the goods while guiding them over a roller system, the material is impregnated with an acidic solution and squeezed out again between rollers. This second squeezing has to be carried out with a roller pressure as low as possible, in order to secure that resulting from the difference between the first and second squeezing a maximum liquid volume is absorbed by the already wet material. The temperature of the acidic impregnation bath should be between 50° and 80° C., so that the splitting and coupling process is instantaneous. The content of the compound having an acidic reaction has to be kept at a level which ensures neutralization of the alkali applied to the textile material together with the coupling component in the alkaline impregnation process, as well as a pH value of from 3 to 7 of the material to be dyed. After the impregnation with the hot acidic solution, the textile material is rinsed hot or cold and finally washed with alkaline baths, rinsed again and dried.

In the process of the invention, the water-insoluble azo dyestuff is produced on the cellulosic fibre portion giving

high colour yields and clear shades. The dyeings obtained have very good fastness properties.

Examples of the textile material to be dyed are mixtures containing between 25% of polyester and 75% of cellulosic fibres, and 70% of polyester and 30% of cellulosic fibres.

Suitable polyester fibres in the blend are fibres made from aromatic polyesters, for example from terephthalic acid or diphenyl-4,4'-dicarboxylic acid and alkane diols or 1,4-cyclohexane-di-methanol, as well as consisting of triacetyl cellulose. The cellulosic fibre portion may be of natural or regenerated origin.

Examples of the coupling components to be used in the process of the invention are especially aromatic o-hydroxy-carboxylic acid arylamides or acylacetic acid arylamides, for example 2,3-hydroxynaphthoic acid arylamides, 6-bromo- or 6-alkoxy-2,3-hydroxynaphthoic acid arylamides or acetoacetic acid arylamides, which have a low to medium substantivity towards cellulosic fibres. When a suitable impregnation equipment is used, for example a small bath tank, also coupling components having a high substantivity towards cellulosic fibres may be used, for example the condensation products from 2,3-hydroxynaphthoic acid and polynuclear, isocyclic and heterocyclic amines, such as aminonaphthalenes, aminocarbazoles or aminodiphenyleneoxides, further heterocyclic o-hydroxy-carboxylic acid arylamides, for example 5 - hydroxy-1,2,1',2' - benzocarbazol - 4 - carboxylic acid arylamides, 2 - hydroxycarbazol - 3 - carboxylic acid arylamides as well as 4,4' - bis - acetoacetylarnino - diphenyls or 2-hydroxyanthracene-3-carboxylic acid arylamides.

As diazoamino or tetrazoamino compounds there are used compounds made from diazotized aromatic or heterocyclic mono- or diamines, for example from diazotized chloroanilines, dichloroanilines, chlorotoluidines, chloranisidines, nitroanisidines, nitrotoluidines, nitroxylidines, nitrophenetidines, cyanotoluidines, cyanoanisidines, aminobenzene-sulfonic acid amides, aminobenzene-carboxylic acid amides, aminophenyl-alkylsulfones, amino-phenyl - arylsulfones or aminophenyl-alkylsulfones, aminodiphenyl ethers, trifluoromethylanilines, mono-acylated phenylenediamines, aminoazobenzenes or 4,4'-diaminodiphenyls, and primary or secondary aliphatic or aromatic amines, for example N-alkylated aliphatic aminocarboxylic acids or aminosulfonic acids, N-alkylated aromatic aminocarboxylic acids, aminosulfonic acids, aminosulfocarboxylic acids or cyanamide.

As anti-diazotates there may be used those compounds which are obtainable from the above-mentioned primary aromatic amines.

Suitable wetting or dispersing agents in the alkaline impregnation bath are condensation products from high-molecular fatty acids and protein degradation products, condensation products from high-molecular fatty acids and aminoalkyl-sulfonic acids as well as purified sulfite-cellulose waste liquor.

The compounds having an acidic reaction used in the acid developing bath may be organic acids, such as formic acid, acetic acid, propionic acid, lactic acid, glycolic acid, tartaric acid or citric acid, or salts having an acidic reaction, such as monosodium phosphate. The acidic developing bath contains also an additional quantity of the sodium salt of the corresponding acid used, so that the pH value can be maintained in a range of from 4 to 6.

As disperse dyestuffs for the pre-dyeing of the polyester fibre portion there may be used such dyestuffs which are suitable for the Thermosol process on account of their thermic properties, i.e. dyestuffs which are capable of

dyeing polyester fibres at temperatures of from 170° to 210° C. and which do not soil the dyeing equipment on account of high volatility. Suitable disperse dyestuffs of this kind from the azo and anthraquinone series are described in Colour Index, Second Edition 1956, vol. 1, pages 1659-1742 and Supplement 1963, pp. S 179-224, as well as in the corresponding additions and amendments, No. 1 (September 1963) to No. 22 (January 1969). When the polyester fibre portion of the mixed fabric is dyed under the conditions of the high-temperature dyeing method (115°-125° C.) or at the boil in a long bath using carriers, also such disperse dyestuffs may be used which have no thermic stability at temperatures of from 170° to 210° C. Suitable disperse dyestuffs for the dyeing of polyester fibres at a temperature of from 100° C. to 125° C. are also described in Colour Index, Second Edition, 1956.

The following example illustrates the invention:

#### Example

A mixed fabric made from 67% of polyethylene glycol terephthalate fibres and 33% of cotton is impregnated with a solution containing, per litre of water of 30° C., 20 g. of Disperse Red 90, and is subsequently squeezed off in such a way that the liquor pick-up amounts to 70% of the dry weight of the goods. Thereafter, the fabric is dried at a temperature of about 100° C., and subsequently passed through a fixation chamber or over hot rollers, so that it is heated for 60 seconds to 180°-210° C. The mixed fabric so pre-dyed is then impregnated at 40°-60° C. with a solution containing, per litre of water, 4 g. of purified sulfite-cellulose waste liquor, 2 g. of a condensation product of oleic acid and methyl taurine, the diazoamino compound obtained from 8.4 g. of diazotized 1 - amino - 2 - methyl - 5 - chlorobenzene and sodium cyanamide, 10 ml. of a 32.5% aqueous sodium hydroxide solution as well as 20 g. of 1 - (2',3' - hydroxynaphthoylamino) - 2 - methoxy - 5 - chlorobenzene, dissolved in 50 ml. of denaturized alcohol, 10 ml. of a 32.5% aqueous sodium hydroxide solution and 50 ml. of water at 40° C.

Subsequently, the fabric is squeezed off to a liquor pick-up of 60% of its dry weight. After the passage through the squeezing rollers, the material is wound up, wrapped in a plastic foil and allowed to dwell in this moist state for an hour at about room temperature, while slowly turning it. The fabric is then passed through a bath containing, per litre of water of 80° C., 90 ml. of a 50% acetic acid, 10 g. of sodium acetate and 50 g. of sodium chloride, and is subsequently squeezed between rollers so that the final liquor pick-up of the goods amounts to 100% of their dry weight. After an air-passage of about 1 minute, the fabric is first passed through a water bath of 60° C., then after-treated at 60° C. and at 95° C. in a further bath containing 1 g. of a reaction product of 10 mols of ethylene oxide with 1 mol of nonylphenol, and 3 g. of sodium carbonate, per litre of water; thereupon it is rinsed and dried. The aftertreatment of the dyed fabric may be also carried out in a bath containing 3 g. of a mixture of 63% of perchloroethylene, 17% of a reaction product of 10 mols of ethylene oxide with 1 mol of nonylphenol and 20% of isopropanol, together with 2 g. of a 25% solution of the sodium salt of nitrilotriacetic acid, per litre of water. An intense red dyeing having good fastness properties is obtained.

The following table lists further coupling components and diazoamino compounds or anti-diazotates that may be used according to the process of the invention, and also disperse dyestuffs for the pre-dyeing of the polyester fibre portion, as well as the shades obtainable therefrom

5  
on mixed fabrics made from 67% of polyethylene glycol  
terephthalate fibres and 33% of cotton:

sufficient to absorb and level the coupling component on  
the fibre.

| Disperse dyestuff                                                           | Coupling component                                                         | Diazoamino compound (DA) or<br>anti-diazotate (AN)                                               | Shade            |
|-----------------------------------------------------------------------------|----------------------------------------------------------------------------|--------------------------------------------------------------------------------------------------|------------------|
| C.I. Disperse Red 82                                                        | 1-(2',3'-hydroxynaphthoylamino)-2-methoxybenzene.                          | DA from diazotized 1-amino-2-methoxy-5-chlorobenzene and sodium N-methylamino acetate.           | Bluish red.      |
| C.I. Disperse Orange 42                                                     | 1-(2',3'-hydroxynaphthoylamino)-2-methylbenzene.                           | DA from diazotized 1-amino-2-methyl-3-chlorobenzene and sodium cyanamide.                        | Yellowish red.   |
| C.I. Disperse Yellow 64                                                     | 4,4'-bis-acetoacetylamino-3,3'-dimethyl-diphenyl.                          | DA from diazotized 1-amino-2-methyl-5-chlorobenzene and sodium N-methylamino acetate.            | Yellow.          |
| C.I. Disperse Blue 79                                                       | 1-(2',3'-hydroxynaphthoylamino)-2-methyl-4-chlorobenzene.                  | DA from diazotized 4,4-diamino-3,3-dimethoxy-diphenyl and N-methyltaurine.                       | Blue.            |
| Do                                                                          | 2-(2',3'-hydroxynaphthoylamino)-naphthalene.                               | DA from diazotized 1-amino-2,5-diethoxy-4-benzoylamino benzene and sodium N-methylamino acetate. | Do.              |
| C.I. Disperse Yellow 64 and C.I. Disperse Blue 35.                          | 1-(2'-hydroxyanthracene-3'-carboylamino)-2-methylbenzene.                  | do                                                                                               | Green.           |
| C.I. Disperse Red 82 and C.I. Disperse Orange 13.                           | 1-(2',3'-hydroxynaphthoylamino)-2,4-dimethoxy-5-chlorobenzene.             | DA from diazotized 1-amino-2-methyl-3-chlorobenzene and sodium cyanamide.                        | Dull bluish red. |
| C.I. Disperse Red 82                                                        | 1-(2',3'-hydroxynaphthoylamino)-2-methoxy-4-chloro-5-methylbenzene.        | AN from diazotized 1-amino-2-methoxy-5-chlorobenzene.                                            | Bluish red.      |
| C.I. Disperse Orange 42                                                     | 1-(2',3'-hydroxynaphthoylamino)-2-methoxybenzene.                          | AN from diazotized 1-amino-2-chloro-5-trifluoro-methylbenzene.                                   | Yellowish red.   |
| C.I. Disperse Orange 13 and C.I. Disperse Blue 56 and C.I. Disperse Red 82. | 1-(2'-hydroxycarbazol-3'-carboylamino)-4-chlorobenzene.                    | DA from diazotized 1-amino-2-methyl-5-chlorobenzene and sodium cyanamide.                        | Brown.           |
| C.I. Disperse Blue 81 and C.I. Disperse Orange 13 and C.I. Disperse Red 82. | 1-(5'-hydroxy-1',2',1",2"-benzocarbazol-4'-carboylamino)-4-methoxybenzene. | DA from diazotized 1-amino-2-methoxy-4-nitrobenzene and sodium cyanamide.                        | Black.           |
| C.I. Disperse Yellow 5 (C.I. 12 790)                                        | 4,4'-bis-acetoacetylamino-3,3'-dimethyl-diphenyl.                          | DA from 1-amino-2-methyl-5-chlorobenzene and sodium cyanamide.                                   | Yellow.          |
| C.I. Disperse Orange 1 (C.I. 11 080)                                        | 1-(2',3'-hydroxynaphthoylamino)-2-methoxybenzene.                          | AN from diazotized 1-amino-2-chloro-5-trifluoromethylbenzene.                                    | Yellowish red.   |
| C.I. Disperse Red 17 (C.I. 11 210)                                          | 2,3-hydroxynaphthoylaminobenzene                                           | DA from diazotized 1-amino-2-methyl-5-chloro-benzene and sodium cyanamide.                       | Red.             |
| C.I. Disperse Blue 9 (C.I. 61 115)                                          | do                                                                         | DA from diazotized 1-amino-2-diethoxy-4-benzoylamino benzene and sodium N-methylaminoacetate.    | Blue.            |

We claim:

1. In a process for the semi-continuous dyeing of textile material made from mixtures of polyester and cellulosic fibres wherein the polyester fibre portion has been predyed with disperse dyestuffs by impregnating said textile material with an alkaline solution containing a substantive coupling component, a diazoamino or tetraazamino compound or an anti-diazotate derived from a primary aromatic amine, and a wetting or dispersing agent, and subsequently developing the dyestuff on the fibre by hot acid treatment, the improvement which comprises treating the alkaline-impregnated textile material, without intermediate drying, with an aqueous solution containing the acidic developing agent at a temperature of from 50° to 80° C. and a pH value of from 3 to 7.

2. A process as claimed in claim 1, wherein the impregnation of the textile material with the alkaline solution is carried out giving a low liquor pick-up of the textile material.

3. A process as claimed in claim 1, wherein the impregnation of the textile material with the alkaline solution is carried out at a temperature of from 30° to 60° C.

4. A process as claimed in claim 1, wherein after the alkaline impregnation the textile material is exposed to an air passage or is wound up and dwelled moist for a time

5. A process as claimed in claim 1, wherein the acidic agent is an organic acid or monosodium phosphate thereof.

35 6. A process as claimed in claim 1, wherein the wetting or dispersing agent is a condensation product of a high-molecular fatty acid and a protein degradation product, or of a high-molecular fatty acid and an aminoalkyl sulfonic acid, or a purified sulfite-cellulose waste liquor.

#### References Cited

##### UNITED STATES PATENTS

3,516,780 6/1970 Kirst et al. ----- 8-44  
2,199,233 4/1940 Williams ----- 8-159

##### FOREIGN PATENTS

413,257 10/1932 Great Britain ----- 8-44

##### OTHER REFERENCES

50 Wygand, Am. Dye. Rep., December 1964, pp. 106-109.  
DuPont, Dyes and Chem. Tech. Bull., vol. 19, No. 2, October 1963, pp. 103-106.

GEORGE F. LESMES, Primary Examiner

55 P. C. IVES, Assistant Examiner

U.S. Cl. X.R.